# EUROPEAN PATENT SPECIFICATION

(11) **EP 0 227 874 B1**
(45) Date of publication and mention of the grant of the patent: **26.09.1990**
(21) Application number: 86100043.8
(22) Date of filing: 03.01.1986
(51) Int. Cl.: G03G 9/08

(54) **Toner for developing electrostatic latent images**
Toner für die Entwicklung elektrostatischer latenter Bilder
Toner pour le développement d'images électrostatiques latentes

(43) Date of publication of application: 08.07.1987
(73) Proprietor: ORIENT CHEMICAL INDUSTRIES, LTD., Osaka-shi (JP)
(72) Inventor: Kawagishi, Yoji, Yawata-shi Kyoto-fu (JP); Narita, Shinichi, Kawachinagano-shi Osaka-fu (JP); Kiriu, Takashi, Osaka-shi (JP); Uomoto, Kenji, Takatsuki-shi Osaka-fu (JP)
(74) Representative: Liedl, Gerhard, Dipl.-Phys.

(56) References cited:
- DE-A- 2 815 857
- DE-A- 3 144 017
- DE-A- 3 329 252

## Description

The present invention relates to a negatively chargeable toner of the dry type for developing electrostatic latent images in electrophotography, electrostatic recording, electrostatic printing as claimed in Claim 1.

Electrostatic latent images can be developed into visible images with a toner which is caused to adhere to the image by electrostatic attraction. Besides liquid developers, powder developers are widely used for developing electrostatic latent images.

The powder developers are divided generally into two types: two-component developers comprising a toner having a mean particle size of 15 J.lm and a carrier of finely divided iron or ferrite mixed with the toner and 100 to 200 µm in particle size, the toner being composed of a natural resin or synthetic resin and a coloring agent, charge control agent, fluidizing agent, etc. dispersed in the resin; and one-component developers comprising a natural resin or synthetic resin, and a coloring agent, charge control agent, fluidizing agent and magnetic material which are dispersed in the resin.

With the two-component developer, the toner is triboelectrically charged by the carrier and deposited on electrostatic images for development. The one-component developers heretofore known include toners which are chargeable by friction with a brush- or plate-like friction member serving the function of the carrier as a substitute therefor. Also made known in recent years is a toner which is chargeable by friction with a finely divided magnetic material which is maintained in a dispersed state. These developing toners are held positively or negatively charged in accordance with the polarity of the electrostatic latent image to be developed.

In order to hold the toner charged, it has been proposed to make use of the triboelectric properties of the resin which is the main component of the toner. With this method, however, the toner is given only a small amount of charge, has great solid surface resistance and therefore produces toner images which are prone to fogging and indistinct. Accordingly, to impart the desired triboelectric chargeability to the toner, dyes and pigments for giving charges and further charge control agents are admixed with toners. Such agents presently used in the art include oil-soluble Nigrosine dyes, etc. for giving positive charges to the toner as disclosed in Published Examined Japanese Patent Application SHO 41-2427, and metal-containing complex salt dyes, etc. disclosed in Published Examined Japanese Patent Application SH045-26478, etc. and adapted to give negative charges to the toner.

Nevertheless, these dyes and pigments as charge control agents are complex in structure and low in stability. They are susceptible to decomposition or degradation to lose charge control properties, owing for example to mechanical friction and impact, changes of temperature and humidity, electrical impact, irradiation with light, etc. Further one of their substantial defects is that these agents are colored substances and are therefore in conflict with the requirement that a colorless or substantially colorless charge control agent should be used for a toner having a particular color.

Although Published Unexamined Japanese Patent Applications SHO 53-127726, SHO 57-104940, SHO 57-111541, SHO 57-124357, etc. disclose various complex compounds which meet this requirement, these compounds still invariably have some slight color.

The document DE-A 3 144 017 describes a toner containing a resin and, as a charge control agent, a Cr, Co or Fe complex of a substituted salicylic acid and of another aromatic hydroxycarboxylic acid having or not having a substituent. The metal complex is reported to have good compatibility with the resin component, to be substantially colorless, and to impart outstanding durability to the toner.

The document DE-A 3 329 252 describes a toner containing an amorphous polyester having an acid number of 10 to 100 and being obtained by reacting an etherified diphenol with a benzene dicarboxylic acid or a mixture of benzene dicarboxylic acids, and a salicylic acid metal complex. The diphenol is either propoxylated or propoxylated and ethoxylated, wherein the content of propoxy groups is not less than 50 mole percent of the total content of the propoxy and ethoxy groups, and the benzene dicarboxylic acid or the mixture of benzene dicarboxylic acids contains up to 40 mole percent of a tribasic or higher-basic aromatic carboxylic acid. The metal complex is reported to react with and cross-link the polyester to improve the viscosity at melt and to prevent adhering of the toner to hot rollers during a fixing process. The addition of charge control agents such as metal-containing dyes and Nigrosin is described as being optional.

The metal complex may be selected from zinc salicylate, chromium salicylate, manganese salicylate, nickel salicylate, cobalt salicylate, cobalt-t-butyl salicylate, chromium-3,5-di-t-butyl salicylate and nickel-3,5-di-t-butyl salicylate.

The object of the present invention is to provide a toner containing a resin and, as a charge control agent capable of giving negative charges to the toner, a compound which remains thermally stable up to a temperature permitting thorough melting and kneading and which is colorless.

It has been found that zinc complex compounds of aromatic hydroxycarboxylic acids which may have a substituent are excellent as such compounds to accomplish the present invention.

The present invention provides a toner for developing electrostatic latent images, the toner containing a resin and, as a charge control agent, a metal complex of an aromatic hydroxycarboxylic acid having or not having a substituent. The toner is characterized in that the metal complex is a zinc complex, toners being excluded wherein the zinc complex is zinc salicylate and the resin is the specific amorphous polyester described in the document DE-A 3 329 252.

Examples of useful aromatic hydroxycarboxylic acids which may have a substituent and which are capable of forming zinc complex compounds are alkyl(C4-C^{g})salicylic acids, 3,5-dialkyl(C₄-Cs)salicylic acids, 2-hydroxy-3-naphthoic acid, alkyl(C₄-Cs)-2-hydroxy-3-naphthoic acids, 5,6,7,8-tetrahalogen-2-hydroxy-3-naphthoic acids, etc.

The zinc complex compound of the present invention can be prepared by dissolving a suitable hydroxycarboxylic acid in water with addition of a sufficient amount of alkali, adding to the solution a metallic zinc giving agent in the agent-to-acid mole ratio of 1:2, heating the mixture, adjusting the pH of the reaction mixture, filtering off the resulting precipitate, thoroughly wahing the precipitate with water and drying the precipitate.

Presumably, the product is represented by the formula wherein A and A_{'} are the residue of an aromatic hydroxycarboxylic acid which may have a substituent, and M is a counter ion.

The counter ion can be changed by changing the condition for the aftertreatment of the reaction mixture. For example, when the reaction mixture is adjuted to a pH of up to 3, then filtered and thereafter washed until the pH becomes about 6 to about 7, the counter ion is hydrogen ion. If the pH is adjusted to neutrality to alkalinity with an alkali, alkali metal ion is obtained. Further if the mixture is treated with hydrochlorides of various amines, various ammonium salts are obtained.

The complex compound of the formula (I) is incorporated into a toner generally in an amount of 0.1 to 10 parts by weight, preferably 0.5 to 5 parts by weight, per 100 parts by weight of the component resin of the toner.

The toner of the present invention is prepared by admixing the complex compound of the formula (I) with at least one of the resins heretofore known for use in toners, such as styrene resin, styrene-acrylic resin, styrene-butadiene resin, epoxy resin, polyester resin, paraffin wax and the like. The resin to be used is determined in view of adhering properties, preservability, free-flowability, amenability to pulverization, etc. While a wide variety of known dyes and pigments are usable as coloring agents, especially suitable as coloring agents for toners for color copying are, for example, Benzidine Yellow, quinacridone, Copper Phthalocyanine Blue, Copper Phthalocyanine Green, etc.

Although the toner is usually mixed with a carrier to provide a two-component developer, it is of course usable as a one-component developer.

Preparation examples are given below.

### Preparation Example 1

### Synthesis of zinc complex compound of 2-hydroxy-3-naphthoic acid

A 42.2 g quantity of 2-hydroxy-3-naphthoic acid (0.22 mole) was completely dissolved in 500 g of 2.7% aqueous solution of caustic soda, and the solution was heated to about 70_{°} C.

Subsequently, 35.5 g (0.13 mole) of zinc sulfate was dissolved in 100 g of water, and the solution was added dropwise to the above solution over a period of 30 minutes. The resulting mixture was maintained at 70 to 80° C for 2 hours. The mixture was adjusted to a pH of 7.0 ± 0.5, whereupon the reaction was completed. The reaction mixture was filtered hot, and the precipitate was washed with water and dried, giving 47.5 g of a complex compound in the form of pale yellow fine particles. (The complex compound, with Na as counter ion, will hereinafter be referred to as Compound (1).)

### Preparation Example 2

### Synthesis of zinc complex compound of 3,5-di-tert-butylsalicylic acid

A 44.5 g (0.18 mole) quantity of 3,5-di-tert-butylsalicylic acid was completely dissolved in 400 g of 2% aqueous solution of caustic soda, and the solution was heated to about 70_{°} C.

Subsequently, 25.5 g (0.09 mole) of zinc sulfate was dissolved in 100 g of water, and the solution was added dropwise to the above solution over a period of 30 minutes. The mixture was maintained at 70 to 80° C for 2 hours and then adjusted to a pH of 7.0 ± 0.5 to complete the reaction. The reaction mixture was filtered hot. The precipitate was washed with water and dried, affording 43 g of a complex compound in the form of white fine particles (with Na as counter ion, hereinafter referred to as Compound (2)).

### Preparation Example 3

### Synthesis of zinc complex compound of tert-butyl-2-hydroxy-3-naphthoic acid

A 12.2 g (0.05 mole) quantity of tert-butyl-2-hydroxy-3-naphthoic acid was completely dissolved in 200 g of 2% aqueous solution of caustic soda, and the solution was heated to about 70° C. Subsequently, 3.4 g (0.025 mole) of zinc chloride was dissolved in 100 g of water. The solution was added dropwise to the above solution over a period of 30 minutes. The mixture was maintained at 70 to 80_{°} C for 2 hours and then adjusted to a pH of 7.0 ± 0.5 to complete the reaction. The reaction mixture was filtered hot. The precipitate was washed with water and dried, giving 13.1 g of a complex compound in the form of pale yellow fine particles (with Na as counter ion, hereinafter referred to as Compound (3)).

Examples of the invention are given below, in which the parts are by weight.

### Example 1

Polyester resin (ATR-2010, product of Kao Soap Co., Ltd.) 100 parts Blue dye (Valifast Blue 2606, product of Orient Kagaku Kogyo Co., Ltd.) 2 parts Blue pigment (Copper Phthalocyanine) 4 parts Compound (1) 1 part

The above ingredients were premixed uniformly by a ball mill to obtain a premix, which was kneaded in a molten state by heat rolls, then cooled, thereafter crushed by a vibrating mill and further pulverized by an air jet mill. The fine powder obtained was screened to obtain a blue toner 10 to 20 µm in particle size.

Three parts of the toner were admixed with 97 parts of a carrier of finely divided iron to prepare a developer. The amount of initial blow-off charge on the developer was -28.3 µc/g. When the developer was used for the magnetic brush developing process with a commercial selenium drum, sharp blue toner images were obtained free from fog. Even after the toner was used for continuously making 50,000 copies, no reduction was observed in the quality of copies.

### Example 2

Epoxy resin (Epikote 1004, product of Shell Chemical Co. Ltd.) 100 parts Carbon black 6 parts Compound (2) 2 parts

The above ingredients were treated in the same manner as in Example 1 to prepare a black toner.

Three parts of the toner obtained were admixed with 97 parts of a carrier of finely divided iron to prepare a developer. The amount of initial blow-off charge on the developer was -24.1 µc/g. When the developer was used for copying in the same manner as in Example 1, sharp black toner images were obtained free from any fog. The toner exhibited no reduction in the quality of copies even after continuously making 50,000 copies.

### Example 3

Styrene-n-butyl methacrylate copolymer resin (65/35) 100 parts C.I. Solvent Yellow 77 6 parts Compound (1)

The above ingredients were treated in the same manner as in Example 1 to prepare a yellow toner.

Three parts of the toner obtained were admixed with 97 parts of a carrier of finely divided iron to prepare a developer. The amount of initial blow-off charge on the developer was -25.2 ₗicfg. When used for copying in the same manner as in Example 1, the developer produced toner images free from any fog and outstanding in reproducibility of thin lines. The toner exhibited no reduction in the quality of copies even after continuously making 50,000 copies.

### Example 4

Styrene-n-butyl methacrylate copolymer resin (65/35) 100 parts Red dye (Valifast Pink 2310, product of Orient Kagaku Kogyo Co., Ltd.) 8 parts Compound (2) 2 parts

A red toner was prepared from the above ingredients in the same manner as in Example 1. Three parts of the toner obtained were admixed with 97 parts of a carrier of finely divided iron to obtain a developer. The amount of initial blow-off charge on the developer was -22.9 I!c/g. When used for copying in the same manner as in Example 1, the developer produced sharp red toner images free from any fog. The toner exhibited no reduction in the quality of copies even after continuously making 50,000 copies.

### Example 5

Styrene-n-butyl methacrylate copolymer resin (65/35) 100 parts C.I. Solvent Yellow 77 6 parts Compound (3)

A yellow toner was prepared from the above ingredients in the same manner as in Example 1.

Three parts of the toner obtained were admixed with 97 parts of a carrier of finely divided iron to obtain a developer. The amount of initial blow-off charge on the developer was -21.8 µc/g. When used for copying in the same manner as in Example 1, the developer produced sharp yellow toner images free from any fog. The toner exhibited no reduction in the quality of copies even after continuously making 50,000 copies.

## Claims (Claims for the following Contracting State(s) : s: BE, CH, DE, FR, GB, IT, LI, LU, NL)

1. A toner for developing electrostatic latent images, said toner containing a resin and, as a charge control agent, a metal complex of an aromatic hydroxycarboxylic acid having or not having a substituent, characterized in that the metal complex is a zinc complex, toners being excluded wherein the zinc complex is zinc salicylate and the resin is an amorphous polyester having an acid number of 10 to 100 and being obtained by reacting an etherified diphenol with a benzene dicarboxylic acid or a mixture of benzene dicarboxylic acids, the diphenol being either propoxylated or propoxylated and ethoxylated and the content of propoxy groups is not less than 50 mole percent of the total content of the propoxy and ethoxy groups, and the benzene dicarboxylic acid or the mixture of benzene dicarboxylic acids contains up to 40 mole percent of a tribasic or higher-basic aromatic carboxylic acid.

2. A toner according to claim 1, wherein the zinc complex is of an alkyl(C₄ to C₉) salicylic acid, a 3,5-dialkyl(C₄ to Cg) salicylic acid, 2-hydroxy-3-naphthoic acid, an alkyl(C₄ to Cg)-2-hydroxy-3-naphthoic acid or a 5,6,7,8-tetrahalogen-2-hydroxy-3-naphthoic acid.

3. A toner according to claim 1, wherein the toner comprises 0.5 to 5 parts by weight of the zinc complex compound per 100 parts by weight of the resin component of the toner.

## Claims (Claims for the following Contracting State(s) : AT)

1. A method for preparing a toner for developing electrostatic latent images by admixing a resin, a coloring agent, and, as a charge control agent, a metal complex of an aromatic hydroxycarboxylic acid having or not having a substituent, characterized by using a zinc complex as the metal complex, a method being excluded wherein the zinc complex used is zinc salicylate and the resin used is an amorphous polyester having an acid number of 10 to 100 and being obtained by reacting an etherified diphenol with a benzene dicarboxylic acid or a mixture of benzene dicarboxylic acids, the diphenol being either propoxylated or propoxylated and ethoxylated and the content of propoxy groups is not less than 50 mole percent of the total content of the propoxy and ethoxy groups, and the benzene dicarboxylic acid or the mixture of benzene dicarboxylic acids contains up to 40 mole percent of a tribasic or higher-basic aromatic carboxylic acid.

2. A method according to claim 1, wherein the zinc complex used is of an alkyl(C₄ to Cₛ) salicylic acid, a 3,5-dialkyl(C₄ to Cg) salicylic acid, 2-hydroxy-3-naphthoic acid, an alkyl(C₄ to Cg)-2-hydroxy-3-naphthoic acid or a 5,6,7,8-tetrahalogen-2-hydroxy-3-naphthoic acid.

3. A method according to claim 1, wherein 0.5 to 5 parts by weight of the zinc complex compound are used per 100 parts by weight of the resin component of the toner.

## Patentansprüche (Patentansprüche für folgende(n) Vertragsstaat(en) : BE, CH, DE, FR, GB, IT, LI, LU, NL)

1. Toner zum Entwickeln elektrostatischer latenter Abbildungen, der ein Harz und, als Ladungssteuermittel, einen Metallkomplex einer aromatischen Hydroxycarbonsäure mit oder ohne einem Substituenten enthält, dadurch gekennzeichnet, daß der Metallkomplex ein Zinkkomplex ist, mit Ausnahme von Tonern, in denen der Zinkkomplex Zinksalicylat und das Harz ein amorpher Polyester mit einer Säurezahl von 10 bis 100 ist, der durch die Umsetzung eines veretherten Diphenols mit einer Benzoldicarbonsäure oder einer Mischung von Benzoldicarbonsäuren hergestellt wurde, wobei das Diphenol entweder propoxyliert oder propoxyliert und ethoxyliert ist und der Propoxygruppengehalt nicht weniger als 50 Mol-% des Gesamtgehalts der Propoxy- und Ethoxygruppen beträgt und die Benzoldicarbonsäure oder die Mischung von Benzoldicarbonsäuren bis zu 40 Mol-% einer drei- oder höherwertigen aromatischen Carbonsäure enthält.

2. Toner nach Anspruch 1, bei dem der Zinkkomplex der einer Alkyl(C₄ bis Cg)salicylsäure, einer 3,5-Dialkyl-(C₄ bis Cg)salicylsäure, der 2-Hydroxy-3-naphthoesäure, einer Alkyl(C₄ bis Cg)-2-hydroxy-3-naphthoesäure oder einer 5,6,7,8-Tetrahalogen-2-hydroxy-3-naphthoesäure ist.

3. Toner nach Anspruch 1, bei dem der Toner 0,5 bis 5 Gewichtsteile der Zinkkomplexverbindung pro 100 Gewichtsteile der Harzkomponente des Toners enthält.

## Patentansprüche (Patentansprüche für folgende(n) Vertragsstaat(en) : AT)

1. Verfahren zur Herstellung eines Toners zum Entwickeln elektrostatischer latenter Abbildungen durch Vermischen eines Harzes, eines Farbstoffes und, als Ladungssteuermittel, eines Metallkomplexes einer aromatischen Hydroxycarbonsäure mit oder ohne einem Substituenten, dadurch gekennzeichnet, daß als Metallkomplex ein Zinkkomplex verwendet wird, mit Ausnahme eines Verfahrens, bei dem der verwendete Zinkkomplex Zinksalicylat und das Harz ein amorpher Polyester mit einer Säurezahl von 10 bis 100 ist, der durch die Umsetzung eines veretherten Diphenols mit einer Benzoldicarbonsäure oder einer Mischung von Benzoldicarbonsäuren hergestellt wurde, wobei das Diphenol entweder propoxyliert oder propoxyliert und ethoxyliert ist und der Propoxygruppengehalt nicht weniger als 50 Mol-% des Gesamtgehalts der Propoxy- und Ethoxygruppen beträgt und die Benzoldicarbonsäure oder die Mischung von Benzoldicarbonsäuren bis zu 40 Mol-% einer drei- oder höherwertigen aromatischen Carbonsäure enthält.

2. Verfahren nach Anspruch 1, bei dem der verwendete Zinkkomplex der einer Alkyl(C₄ bis C₉)salicylsäure, einer 3,5-Dialkyl-(C₄ bis Cg)salicylsäure, der 2-Hydroxy-3-naphthoesäure, einer Alkyl(C₄ bis Cg)-2-hydroxy-3-naphthoesäure oder einer 5,6,7,8-Tetrahalogen-2-hydroxy-3-naphthoe- säure ist.

3. Verfahren nach Anspruch 1, bei dem 0,5 bis 5 Gewichtsteile der Zinkkomplexverbindung pro 100 Gewichtsteile der Harzkomponente des Toners verwendet werden.

## Revendications (Revendications pour l'(les) Etat(s) contractant(s) suivant(s) : BE, CH, DE, FR, GB, IT, LI, LU, NL)

1. Un toner pour le développement d'images électrostatiques latentes, ledit toner contenant une résine et, en tant qu'agent de commande de charge, un complexe métallique d'un acide hydroxycarboxylique aromatique ayant ou n'ayant pas un substituant, caractérisé en ce que le complexe métallique est un complexe de zinc, les toners, dont sont exclus ceux dans lesquels le complexe de zinc est du salicylate de zinc et la résine est un polyester amorphe présentant un indice d'acidité de 10 à 100, étant obtenus par réaction d'un diphénol éthérifié avec un acide dicarboxylique benzène ou un mélange d'acides dicarboxyliques benzène, le diphénol étant soit propoxylé, soit propoxylé et éthoxylé, et la teneur en groupes propoxy n'étant pas inférieure à 50 moles pour-cents de la teneur totale en groupes propoxy et éthoxy, et l'acide dicarboxylique benzène ou le mélange d'acides dicarboxyliques benzène contient jusqu'à 40 moles pour-cents d'un acide carboxylique aromatique tribasique ou plus que tribasique.

2. Un toner selon la revendication 1, dans lequel le complexe de zinc est un acide salicylique alkyle (C₄ à Cₛ), un acide salicylique 3,5-dialkyle (C₄ à Cₛ)-2-hydroxy-3-naphtoïque, un acide alkyle (C₄ à Cₛ)-2-hydroxy-3-naphtoïque ou un acide 5,6,7,8-tétrahalogène-2-hydroxy-3-naphtoïque.

3. Un toner selon la revendication 1, comportant de 0,5 à 5 parties en poids du composé complexe de zinc pour 100 parties en poids du constituant résine du toner.

## Revendications (Revendications pour l'(les) Etat(s) contractant(s) suivant(s) : AT)

1. Un procédé de préparation d'un toner pour le développement d'images électrostatiques latentes par mélange d'une résine, d'un agent colorant et, en tant qu'agent de commande de charge un complexe métallique d'un acide hydroxycarboxylique aromatique ayant ou n'ayant pas un substituant, caractérisé par l'utilisation d'un complexe de zinc en tant que complexe métallique, le procédé, à l'exclusion de celui dans le complexe de zinc et la résine utilisée est un polyester amorphe présentant un indice d'acidité de 10 à 100, étant obtenu par réaction d'un diphénol éthérifié avec un acide dicarboxylique benzène ou un mélange d'acides dicarboxyliques benzène, le diphénol étant soit propoxylé, soit propoxylé et éthoxylé, et la teneur en groupes propoxy n'étant pas inférieure à 50 moles pour-cents de la teneur totale en groupes propoxy et éthoxy, et l'acide dicarboxylique benzène ou le mélange d'acides dicarboxyliques benzène contient jusqu'à 40 moles pour-cents d'un acide carboxylique aromatique tribasique ou plus que tribasique.

2. Un procédé selon la revendication 1, dans lequel le complexe de zinc utilisé est un acide salicylique alkyle (C₄ à Cₛ), un acide salicylique 3,5-dialkyle (C₄ à Cₛ), un acide 2-hydroxy-3-naphtoïque, un acide alkyle (C₄ à C₉)-2-hydroxy-3-naphtoïque ou un acide 5,6,7,8-tétrahaiogène-2-hydroxy-3-naphtoïque.

3. Un procédé selon la revendication 1, dans lequel on utilise de 0,5 à 5 parties en poids du composé complexe de zinc pour 100 parties en poids du constituant résine du toner.
